

Nov. 15, 1938.

F. R. HENSEL ET AL

2,136,918

COPPER ALLOYS

Filed Sept. 15, 1937



INVENTORS  
Franz R. Hensel  
By Earl J. Larsen  
Bartholin  
ATTORNEY

## UNITED STATES PATENT OFFICE

2,136,918

## COPPER ALLOYS

Franz R. Hensel and Earl I. Larsen, Indianapolis,  
Ind., assignors to P. B. Mallory & Co., Inc., In-  
dianapolis, Ind., a corporation of Delaware

Application September 15, 1937, Serial No. 164,039

1 Claim. (Cl. 75—154)

This invention relates to copper alloys.

An object of the invention is to produce an improved copper base alloy.

Another object is to produce a copper-tin base alloy which can be age hardened.

Other objects of the invention will be apparent from the following description taken in connection with the appended claim.

The present invention comprises the combination of elements, methods of manufacture and the product thereof, brought out and exemplified in the disclosure hereinafter set forth, the scope of the invention being indicated in the appended claim.

15 In the drawing:

Figure 1 is a graph having curves, illustrating the improvement in the hardness and electrical conductivity of the alloy of the present invention during age hardening;

20 Figure 2 is a graph showing the effect of cold working after quenching from high temperatures and subsequent aging at a temperature of 450 degrees C.; and

25 Figure 3 is a graph showing the effects of cold working the quenched and aged alloy.

While a preferred embodiment of the invention is described herein, it is contemplated that considerable variation may be made in the method of procedure and the combination of elements, without departing from the spirit of the invention.

30 Copper-tin alloys are frequently used at the present time for the purpose of current carrying springs, special trolley wires and electrical conductors of various types. These alloys, while having numerous advantages, when used at low temperatures, are not entirely satisfactory when used at even moderately high temperatures, such as 300-350 degrees C. Furthermore, in order to obtain a reasonably high hardness, it is necessary to add a tin content ranging from 5-10%. This high percentage of tin, which is held in solid solution by the copper decreases the electrical conductivity enormously.

45 According to the present invention, copper-tin base alloys are improved by the addition of zirconium. The improved alloys can not only be made of greater hardness than prior copper-tin alloys, but are also capable of retaining their hardness at high temperatures.

50 According to the preferred method of carrying out the present invention, an alloy is made containing copper, tin and zirconium in substantially the following proportions:

|           | Per cent |
|-----------|----------|
| Tin       | 0.1-10   |
| Zirconium | 0.05-5   |
| Copper    | Balance. |

It is possible likewise to improve the characteristics of other copper-tin alloys by the addition

of zirconium, particularly copper-tin alloys containing small percentages of phosphorus. Such alloys are generally known as phosphor bronzes and usually contain from about 0.01 to 1.0% phosphorus. In general, copper-tin base alloys, containing small proportions of silver, zinc, magnesium, calcium, lithium, silicon, beryllium, cadmium, iron, nickel, cobalt, manganese, can be improved by the addition of zirconium in substantially the proportions indicated above.

5 The addition of zirconium to the above alloys renders them susceptible to age hardening.

The alloy can be made according to standard alloying methods, such as melting the copper and adding the desired amount of tin. Afterwards 15 the zirconium may be introduced in any suitable form, such as pure zirconium wrapped in foil, or a hardener alloy or zirconium powder mixed with copper powder and compressed to a high density.

After the alloy has been prepared according to 20 the standard alloying methods, the heat treatment may be carried out as follows:

The alloy in the form of a billet or a sand casting or any other desired form, is raised in temperature to above 700 degrees C. The alloy 25 is then quenched from this high temperature and subsequently aged at temperatures below 700 degrees C. This heat treatment results in a considerable improvement in the hardness of the alloy. For example, an alloy of

|           | Per cent |
|-----------|----------|
| Zirconium | 0.5      |
| Tin       | 0.5      |
| Copper    | Balance. |

having a Rockwell B hardness of 21, after 35 quenching, may be given a Rockwell B hardness of 60 by the heat treating process. This is shown in a curve of Figure 1. Another remarkable effect of the heat treatment is the marked improvement of the electrical conductivity. With 40 the alloy combination of 1/2% tin and 1/2% zirconium an electrical conductivity of 63% was reached.

If a certain amount of cold working is applied after quenching, this same alloy will reach a 45 higher hardness after aging. If it is, for instance, reduced 60% in thickness, the hardness after aging is 79 Rockwell B.

If the alloy is completely age hardened and cold worked afterwards, a Rockwell B hardness 50 of over 70 can be easily obtained with 25% reduction.

In many applications, it is not necessary to retain the high electrical conductivity of 65%, and higher tin contents may be employed. In 55 this case, the increase in hardness is much more pronounced and materials can be produced which are ideally suited for springs. Due to the fact that the material will not anneal until high temperatures are reached, these springs will have 60

a decreased tendency to creep in service and the material may be subjected to higher temperatures than was heretofore possible.

Usually the phosphor bronzes were susceptible to annealing and the annealing temperature was a function of the amount of cold work. In other words, if the material was severely cold worked, the annealing temperature would be comparatively low. With the addition of zirconium, all of these disadvantages are entirely overcome and a material is produced which will not soften until the aging temperature is reached. Furthermore, if the material has been softened, its hardness can be restored by a heat 10 treating process. This is very important, because in some cases, the metal might have been reduced in thickness to the desired dimensions and further reductions are undesirable. In such cases an ordinary phosphor-copper spring would 15 be useless, whereas the present invention provides a new means of restoring hardness as well as improved electrical characteristics. The addition of zirconium further produces a material which will have a very fine grain size and will 20 retain this grain size even during the annealing operations which are necessary in the manufacturing process.

The alloys have a high resistance to corrosion and a reduced tendency to oxidation.

30 The alloys are well suited for any electrical or mechanical use at room temperatures and also at elevated temperatures, since the physical properties and electrical properties are main-

tained at such elevated temperatures for indefinite periods.

The alloys are also suited for the manufacture of bronze castings which may be used for such applications as commutator segments, collector 5 rings, structural parts of electrical machinery.

In addition, the alloys are well suited for welding electrode tips as used in resistance welding and for welding wheels.

Another important use of these high strength 10 alloys is in the manufacture of parts used for internal combustion engines where high heat conductivity is needed in combination with high strength.

While the present invention as to its objects 15 and advantages has been described herein, as carried out in specific embodiments thereof, it is not desired to be limited thereby, but it is intended to cover the invention broadly, within the spirit and scope of the appended claim.

What is claimed is:

An age-hardened alloy containing about 0.1 to 10% tin, about 0.05 to 5% zirconium, and the balance substantially all copper, characterized by a combination of high hardness and high 25 electrical and heat conductivity and further characterized by the fact that its hardness and conductivity is not permanently adversely affected by temperatures in the order of 400-450 degrees C.

FRANZ R. HENSEL.  
EARL I. LARSEN.